

# UNITED STATES PATENT OFFICE.

JESSE B. BRONSTEIN AND CHARLES E. WALLER, OF ALLENTOWN, PENNSYLVANIA,  
ASSIGNORS TO INDEPENDENT NON-FREEZING POWDER COMPANY, OF NEWARK,  
NEW JERSEY, A CORPORATION OF NEW JERSEY.

## NITRO-STARCH EXPLOSIVE.

1,188,245.

Specification of Letters Patent. Patented June 20, 1916.

No Drawing.

Application filed July 1, 1914. Serial No. 848,476.

To all whom it may concern:

Be it known that we, JESSE B. BRONSTEIN and CHARLES E. WALLER, citizens of the United States, and residents of Allentown, 5 Lehigh county, Pennsylvania, have invented certain Improvements in Nitro-Starch Explosives, of which the following is a specification.

Our invention relates to nitro-starch explosives.

Heretofore, nitro-starch explosives have been made containing nitro-starch as the explosive base (and in using the term "nitro-starch explosives" we refer to explosives 15 such as employ nitro-starch as an explosive base and are used for blasting purposes), nitrate of soda as the oxygen carrier and suitable quantities of an anti-acid such as calcium carbonate and of a waterproofing 20 material such as paraffin oil. These powders have been graded to suit conditions encountered in practice, by varying the percentage of nitro-starch and nitrate of soda. In varying the proportions of the nitro- 25 starch and nitrate of soda to secure the different grades, we have found it desirable, in order to avoid undue oxygen excess, to add an additional combustible, preferably carbon or carbonaceous material in some 30 form, and it is the object of our present invention to provide a suitable material for the purpose mentioned.

A further object is to provide a nitro-starch powder having an additional combustible ingredient which will increase both 35 the propellant force and brisance or shattering force of the explosive, without making any material increase in the cost and without any deleterious effect.

40 A carbonaceous material for our purpose must answer several requirements. It must not have the effect of unduly desensitizing. It must be sufficiently susceptible to oxidation. It should be non-hygroscopic, and 45 should be physically coarse and hard.

We have discovered that we can use to 50 excellent advantage for the purpose above referred to, a carbonaceous material consisting of an ordinary cereal such, for example, as wheat, when ground into a coarse, hard and granular form, of such size that the granules will pass through a twenty-mesh screen, but not through a sixty-mesh screen, and having all of the finer particles

separated therefrom. The combustible carbonaceous material which we employ can be obtained as "screenings" from flour and starch mills, or can be specially prepared for use, and we have found that it does not desensitize the explosive as does a finely ground material, and at the same time it is very readily oxidized, is non-hygroscopic and has all of the desired physical characteristics.

55 In order to illustrate the beneficial effects of introducing a proper proportion of this combustible carbonaceous material into nitro-starch explosives which would otherwise contain a considerable oxygen excess, it may be stated that we have ascertained by experiment that the addition of 6 per cent. of this material into an explosive containing 30 per cent. of nitro-starch has the effect of increasing the propellant force, as indicated by the ballistic mortar, about 10 per 75 cent.

An illustration of one explosive mixture employing the carbonaceous material referred to may be given as follows:

|                       |       |        |
|-----------------------|-------|--------|
| Nitro-starch          | 26.0% | 80     |
| Nitrate of soda       | 64.6% |        |
| Carbonaceous material | 8.0%  |        |
| Paraffin oil          | .4%   |        |
| Calcium carbonate     | 1.0%  | 85     |
|                       |       | 100.0% |

We have successfully used mixtures containing as high as ten per cent. by weight of the said carbonaceous material.

90 While the formula above given can be successfully used for some purposes, experiment has shown that the brisance or shattering force of the explosive is not increased by the addition of the carbonaceous material to the same extent as the propellant force. It is desirable for most purposes 95 that the "shattering force" should increase proportionately with the "propellant force," and we have discovered that within certain limits, the use of small amounts of sulfur, together with the carbonaceous material will secure the desired increase in the shattering force. When using both ingredients, to wit, the carbonaceous material referred to, and sulfur, we prefer to use them in about equal parts, and it is also best to so proportion 100 the two ingredients to the remainder of the

ingredients as to cause the oxidizing elements to just balance with the amount of available oxygen; that is to say, so that there shall be no excess oxygen upon explosion.

An illustration of a mixture in which we have successfully used carbonaceous material and sulfur is as follows:

|                       |        |
|-----------------------|--------|
| Nitro-starch          | 30 %   |
| 10 Sodium nitrate     | 58.0%  |
| Calcium carbonate     | 1.5%   |
| Paraffin oil          | 0.5%   |
| Carbonaceous material | 5.0%   |
| Sulfur                | 5.0%   |
| 15 Total              | 100.0% |

15 Total 100.0%

To further explain the effect of the carbonaceous material and the sulfur, it may be stated, that the presence of the carbonaceous material tends to increase the gaseous products of explosion, while the presence of sulfur tends to increase the temperature of explosion. The presence of sulfur in the 25 quantities in which we use this ingredient also tends to increase the sensitiveness of the explosive. Neither of the materials tends in any way to reduce the stability of the explosive, nor do said materials have 30 any injurious effect on the physical condition of the explosive. In short, the introduction of these ingredients in the proportions in which we use them, tends to materially increase both the propellant force 35 and brisance of the explosive without making any material increase in the cost of the explosive and without having any injurious effect.

In the instance given the propellant force 40 and the shattering force are so proportioned one to the other as to give the best results in all that class of work which involves moving great masses of rock in very large quantities. This class of work is exemplified in 45 any of the large quarry or excavation operations where blasts comprising thousands of pounds of explosives are frequently made and where thousands of tons of stone are brought down with each blast. In such work 50 in order to get the best results from the energy of the explosive, it is necessary that neither the shattering force nor the propellant force of the explosive be unduly preponderant. For instance, if the explosive 55 has too great a brisance or shattering force, too large a proportion of its total energy is consumed in pulverizing and burning the rock in immediate contact with the charge, thus resulting not only in a useless waste of 60 energy, but also having another bad effect, in that under these conditions the charge chamber is instantaneously enlarged at the moment of explosion, before the main mass of rock or earth begins to move and before 65 the gases have developed their full pressure,

with the result that the gases when they do reach their maximum pressure must act in an enlarged chamber, thereby causing a reduction of the pressure per unit of area. On the other hand, if too large a proportion of the energy of the explosive is developed as propellant force, the rock is thrown out in great masses, which are difficult to handle in quarry or excavation operations. It is for this reason that in ordinary cases we 75 prefer to balance the propellant and shattering forces by employing the carbonaceous material and sulfur in substantially equal proportions. It is to be understood, however, that we do not wish to confine ourselves, in this aspect of our invention, to the use of the two ingredients in equal proportions, as in some cases the advantages of our invention or some of them can be secured by the employment of either ingredient in lesser proportion than the other.

It will also be understood that the shattering force and propellant force of the explosive can be varied in ratio otherwise than by a mere variation of the proportions of carbonaceous material and sulfur employed. For example, we have found that other ingredients, such as barium nitrate, may be substituted for a portion of the sodium nitrate employed as the oxygen carrier, with the result of greatly increasing the shattering force of the explosive. We do not, however, in this application, claim this feature as part of our present invention, as the same has been made, or is about to be made, the subject of another application. It is also to be understood that in the broader aspect of our invention, we do not wish to be confined to the employment of the described carbonaceous material, with 90 or without sulfur, solely for the purpose of overcoming an oxygen excess due to the particular proportions of nitro-starch and nitrate of soda employed in the mixture, as said carbonaceous material, or carbonaceous material and sulfur, can be usefully employed in nitro-starch powders where oxygen excess is due to other causes. For example, in our application filed August 7, 1913, Serial No. 783,601, we have described 95 the use of a mixture of nitrate of ammonia and trinitrotoluene as a substitute for a portion of the nitro-starch in nitro-starch explosives, and in certain cases such substitution leads to undue oxygen excess, and our present invention may be very usefully employed in mixtures in which the nitrate of ammonia and trinitrotoluene are also employed.

110 As this application possesses matter in common with an application filed by us August 7, 1913, Serial No. 783,601, it is to be treated as a continuation of said prior application as far as the common subject-matter is concerned.

70

75

80

85

90

95

100

105

110

115

120

125

130

We claim:

1. A detonating explosive containing nitro-starch as an explosive base, and combustible carbonaceous material comprising cereal screenings in the form of hard granules; said carbonaceous material not exceeding substantially ten per cent. (10%) by weight of the entire explosive.
2. A detonating explosive containing nitro-starch as an explosive base, an oxygen carrier in such proportion to said nitro-starch as to result in oxygen excess, and combustible carbonaceous material comprising cereal screenings in the form of hard granules.
3. A detonating explosive containing nitro-starch as an explosive base, an oxygen carrier in such proportion to said nitro-starch as to result in oxygen excess, and combustible carbonaceous material comprising cereal screenings in the form of hard granules; such carbonaceous material being proportioned to properly balance the oxygen content of the mixture.
4. A detonating explosive containing nitro-starch as an explosive base, combustible carbonaceous material comprising cereal screenings in the form of hard granules, and sulfur.
5. A detonating explosive containing nitro-starch as an oxygen carrier in such proportion to said nitro-starch as to result in oxygen excess, combustible carbonaceous material comprising cereal screenings in the form of hard granules, and sulfur; the carbonaceous material and sulfur being proportioned to properly balance the oxygen content of the mixture.

tro-starch as an explosive base, an oxygen carrier in such proportion to said nitro-starch as to result in oxygen excess, combustible carbonaceous material comprising cereal screenings in the form of hard granules, and sulfur.

6. A detonating explosive containing nitro-starch as an explosive base, an oxygen carrier in such proportion to said nitro-starch as to result in oxygen excess, combustible carbonaceous material comprising cereal screenings in the form of hard granules, and sulfur; the carbonaceous material and sulfur being proportioned to properly balance the oxygen content of the mixture.

7. A detonating explosive containing nitro-starch as an explosive base, combustible carbonaceous material comprising cereal screenings in the form of hard granules, and sulfur; the carbonaceous material and sulfur being used in substantially equal parts by weight.

In testimony whereof, we have signed our names to this specification, in the presence of two subscribing witnesses.

JESSE B. BRONSTEIN.  
CHARLES E. WALLER.

Witnesses:

M. ELEANOR ROBERTS,  
Jos. H. KLEIN.

Copies of this patent may be obtained for five cents each, by addressing the "Commissioner of Patents, Washington, D. C."